

S. A. FLOWER, DEC'D.  
C. E. FLOWER, ADMINISTRATOR.  
PROCESS FOR MAKING A RESILIENT FIBER.  
APPLICATION FILED OCT. 10, 1907.

957,152.

Patented May 3, 1910.



Witnesses  
Martin Jimansky  
Sigmund Schuler

By his Attorney *Samuel A. Flower*  
*Atde Bourneville*

# UNITED STATES PATENT OFFICE.

SAMUEL A. FLOWER, OF NEW YORK, N. Y.; CHARLES E. FLOWER ADMINISTRATOR OF  
SAID SAMUEL A. FLOWER, DECEASED.

## PROCESS FOR MAKING A RESILIENT FIBER.

957,152.

Specification of Letters Patent.

Patented May 3, 1910.

Application filed October 10, 1907. Serial No. 396,841.

*To all whom it may concern:*

Be it known that I, SAMUEL A. FLOWER, a citizen of the United States, and a resident of the borough of Manhattan, in the county of New York and State of New York, have invented certain new and useful Improvements in Processes for Making a Resilient Fiber, of which the following is a specification.

10 This invention relates to a process for making resilient fiber which is specially applicable to a lubricating packing, but can be used for other purposes. Its object specifically is the process to make a fiber which will have the requisite resilience to maintain a fibrous conductor in continuous contact with the object, like a journal that is to be lubricated. To produce the resilient fiber, a vegetable fiber, like coir fiber is treated 20 for about thirty minutes in a bath of caustic soda of about 30° Baumé which produces an alkaline lignin, curling the fiber and making it resilient. The fiber is then placed in a bath of acetic acid of 1° Baumé for about 25 twenty minutes which neutralizes any excess of alkali present. Next it is treated in a bath of anilin, composed of one part of anilin and five hundred parts of water to set the fiber, after which the said fiber is dried 30 by heat when used for a lubricating packing.

By the terms set the fiber or setting the fiber as used in the specification and claims is meant giving fixed form to the fiber.

The prepared fiber as just described is 35 mixed in a picker with cotton yarn and wool yarn in the following proportions: twenty per cent. of the coir fiber, forty five per cent. cotton yarn, and thirty five per cent. wool yarn.

40 In the accompanying drawing the coir fiber is shown at 10, and the cotton yarn and wool yarn at 11 and 12 respectively.

The packing may be modified by mixing the coir fiber with either cotton yarn or wool yarn, thereby omitting one of the latter elements. The packing is specially applicable for journal boxes of car axles.

Having described my invention, I claim:

1. The process of making a resilient fiber consisting in treating a vegetable fiber to 50 an alkali to make it resilient, neutralizing any excess of alkali present by an acid solution, then setting the fiber in a bath of anilin, and finally drying the product.

2. The process of making a resilient fiber 55 consisting in treating coir fiber to an alkali to make it resilient, next neutralizing any excess of alkali present by an acid solution, then setting it in a bath of anilin and finally drying the product.

3. The process of making resilient fiber 60 consisting in treating a vegetable fiber in a bath of caustic soda to make it resilient, next neutralizing any excess of alkali present in a solution of acetic acid, then setting 65 the fiber in a bath of anilin and finally drying the product.

4. The process of making a resilient fiber for lubricating packing consisting in treating coir fiber in a bath of caustic soda to 70 make the fiber resilient, neutralizing any excess of alkali present in a bath of acetic acid, then setting the fiber in a bath of anilin and finally drying the product.

Signed at the borough of Manhattan in 75 the county of New York, and State of New York, this 8th day of October A. D. 1907.

SAMUEL A. FLOWER.

Witnesses:

SIGMUND SCHULER,  
MARTIN ZIMANSKY.